

F. RUDOLPH.

SHEET METAL CONTAINER FOR THE PRESERVATION OF FOOD.

APPLICATION FILED MAR. 9, 1914.

1,206,379.

Patented Nov. 28, 1916.



Fig. 2



Witnesses:

Wm. Gaige  
Joseph Harris

Inventor

Franklin Rudolph  
By Munday, Earle, Adcock  
& Clarke  
his Atty.

# UNITED STATES PATENT OFFICE.

FRANKLIN RUDOLPH, OF CHICAGO, ILLINOIS, ASSIGNOR TO AMERICAN CAN COMPANY, OF NEW YORK, N. Y., A CORPORATION OF NEW JERSEY.

## SHEET-METAL CONTAINER FOR THE PRESERVATION OF FOOD.

1,206,379.

Specification of Letters Patent.

Patented Nov. 28, 1916.

Application filed March 9, 1914. Serial No. 823,333.

To all whom it may concern:

Be it known that I, FRANKLIN RUDOLPH, a citizen of the United States, residing in Chicago, in the county of Cook and State of Illinois, have invented a new and useful Improvement in Sheet-Metal Containers for the Preservation of Food, of which the following is a specification.

This invention relates to an improvement 10 in sheet metal containers for the preservation of food and the invention consists in lacquering the interior of the can with a multiplicity of coatings to adapt it to resist the destructive action of contents of different kinds.

In the accompanying drawing which forms a part of this specification, Figure 1 is a diagrammatic view of an ordinary sheet metal can or container such as is used in the 20 preservation of various food products as fish, beets, vegetables. Fig. 2 is an enlarged, fragmentary section of any one of the walls of the container or of the two ends thereof to illustrate the use of the multiplicity of lacquerings or coatings.

One of the most serious difficulties encountered in the manufacture of sheet metal food containing cans in which to pack and preserve food by the process of sterilization by heat, has been the fact that in some 30 cases the food contents has an acid reaction, for example, and in other cases, an alkaline reaction and in still other cases a different chemical corrosive effect upon the interior

35 of the can. It has been found necessary in many cases to protect the interior of the sheet metal vessel by a coating to guard against the formation of poisonous salts of tin due to the chemical action of the contents upon the tin coating of the sheet metal vessel. Thus the interior of tin cans has been lacquered or varnished by lacquers of various kinds. But it has been found that these lacquers do not always protect the tin 40 coating from the action of the contents and special provision is required to be made by the use of some particular kind of lacquer or coating in connection with different kinds of contents and sometimes, as 45 in the case of shrimps, crabs, lobsters, it has

been found necessary to protect the lacquer by inclosing the contents in parchment or cloth cases within the can.

The present invention consists in coating the interior of the tin sheet metal vessel or 55 container with a multiplicity of coatings, each of a different character and adapted to resist a different chemical action. Thus, for example, to illustrate my invention and enable others to practice the same, I coat the 60 interior of the tin can first with a lacquer consisting of any of the suitable varnish gums held in solution in benzol and bake the same on in the ordinary way. Thereafter, when this coating is dry and hard I apply 65 a second coating consisting, for example, of shellac in an alcoholic solution which I spray upon the interior of the lacquered or coated can. The result is, a can which will resist all of the kinds of contents that may 70 be resisted by the shellac coating and all of the kinds of contents that may be resisted by the baked on coating. Moreover, in addition to this, the double coating also tends to cover up any defects that may exist in 75 either one of the coatings.

The utility of the container is thus greatly enhanced while its expense of manufacture is not materially increased.

In the illustrative section at Fig. 2, A is 80 the sheet of iron provided with a coating B of tin on each side thereof, C represents the baked on lacquer with a benzol solvent and D represents the sprayed on lacquer with the alcoholic solvent, the whole representing 85 a fragmentary section of the form of the invention used herein to illustrate the same.

I hereby disclaim as not of my invention the aluminum lined can shown and described in the Norton Patent #863,086 90 dated August 13, 1907.

I claim:

1. A sheet metal container the interior of which is provided with two lacquer coatings, the first coating being baked on to the 95 tinned surface of the container and the second coating being sprayed on to and adherent to the first coating, the first of said coatings consisting of varnish gum, and the second of said coatings consisting of shellac, 100

the said two coatings being of different resistant qualities.

2. A sheet metal tin coated container comprising on the interior tinned surface thereof: first a baked on lacquer coating of one constituency adhering to and covering the inner surface and ends of the container; and second a sprayed on lacquer coating of an-

other constituency adhering to and covering the first named lacquer coating.

Signed this 3d day of March, 1914, in the presence of two subscribing witnesses.

FRANKLIN RUDOLPH.

Witnesses:

H. M. MUNDAY,  
JOSEPH HARRIS.